

# UNITED STATES PATENT OFFICE.

OSKAR NAGEL, OF NEW YORK, N. Y.

## PROCESS OF MAKING SPELTER.

SPECIFICATION forming part of Letters Patent No. 699,969, dated May 13, 1902.

Application filed November 13, 1901. Serial No. 82,134. (No specimens.)

*To all whom it may concern:*

Be it known that I, OSKAR NAGEL, a subject of the Emperor of Austria-Hungary, residing in the borough of Manhattan, city of New York, State of New York, have invented a certain new and useful Process of Making Spelter, of which the following is a description.

My invention relates to an improved process for making spelter.

10 The invention has been specially designed for the purpose of providing a process by which spelter can be produced in a blast-furnace with consequent economy in the cost of production; but the invention is not limited 15 to the making of spelter in such an apparatus, but can be carried out in connection with the condensation of zinc-vapors obtained by any other reducing process or reaction—as, for instance, by heating blonde with iron or 20 iron-silicate, ( $Fe_4SiO_6$ .)

I am of course aware that during the past fifty years the possibility of producing spelter in a blast-furnace has been frequently suggested and numerous experiments have 25 been made to accomplish that result; but so far as I know no one prior to myself succeeded in condensing zinc in such an apparatus to a pure liquid mass. In all of the prior attempts to produce spelter in a blast-furnace, so far 30 as I know, the result has been the production of zinc-dust, which, from a metallurgical standpoint, can only be regarded as an intermediate product capable, it is true, of being converted to spelter by further reduction.

35 In experimenting for the purpose of verifying the commonly-accepted explanation of the cause of the production of zinc-dust where the attempt has been made to obtain spelter in a blast-furnace I have found that zinc-vapors, if diluted with indifferent or inactive gases, such as nitrogen, will in every instance condense to dust instead of to liquid spelter, and I have further ascertained that if in addition to such indifferent or inactive gases 40 the zinc-vapors are diluted with oxidizing-gases, such as oxygen or carbonic acid, a corresponding part of the resulting dust will be immediately oxidized. In the prior attempts referred to indifferent and oxidizing 45 gases have been inevitably present, since the reducing operation was always carried on in

the presence of air blown into and through a mixture of ore and coal, coke, or charcoal.

I have discovered that spelter can be made in a blast-furnace if indifferent, inactive, and 55 oxidizing gases are excluded from the evolved vapors, as well in the furnace itself as in the condensing apparatus, by employing only a gas which performs a reducing operation and which passes with the vapors to the condensing apparatus. When such a gas is employed 60 for performing a reducing operation in a blast-furnace, the evolved zinc-vapors will condense to a liquid mass free from dust, the resulting spelter obtained being as pure as that 65 which is now secured in the ordinary processes using retorts and muffles.

The invention consists in subjecting a suitable zinc ore, preferably mixed with coal, to the action of water-gas which is practically 70 free from inert, indifferent, and oxidizing gases, and by which the zinc will be reduced and as an evolved vapor will be condensed in an atmosphere which permits the formation of pure spelter. The active reducing-gas 75 which I employ in my process is advantageously and preferably heated before being injected into the furnace, thereby practically doing away with the necessity of using other fuel and, in consequence, overcoming the 80 greatest difficulty with which prior experimenters met—to wit, the dilution and oxidation of the zinc-vapors by combustion-gases.

In the preferred embodiment of the invention, therefore, the active reducing water-gas, being first heated to the necessary temperature, is injected into the furnace, which is charged with a dry or baked mixture in the proportion of one part of coal and seven parts of roasted blonde, (or the corresponding 90 amount of any oxidic zinc ore, or willemite, or franklinite, or complex blonde, or mixtures of such materials, or, in fact, any zinc-oxid material,) the coal being employed only for the purpose of immediately reducing any gases which 95 become oxidized by the reduction of the zinc oxid. The zinc-vapors thereby obtained are in as concentrated a condition as in the ordinary processes of zinc distillation in muffles or retorts, and the condensation to spelter is 100 readily effected, taking place with a yield of from ninety to ninety-five per cent. of zinc,

containing about .045 per cent. lead and .04 per cent. iron.

In a more specific sense, therefore, the invention consists in injecting heated water-gas into the zinc ore in a blast-furnace and, preferably, for the reasons stated, into a mixture of zinc ore and coal with the reactions indicated.

The gas which I use for reduction and for the atmosphere of condensation is, as stated, water-gas, which contains about equal volumes of carbon monoxid and hydrogen, both of which gases are eminently reducing. The water-gas, which can be cheaply prepared by well-known methods, before being injected into the blast-furnace is first heated in ovens of any desired form, which ovens are heated by the waste reduction-gases (coming from the condensation apparatus) or by producer-gas, which is produced intermediately with the water-gas by well-known methods. The reducing-gas is preferably forced into the furnace by means of a fan or blower the capacity of which is properly calculated to accommodate the desired bulk of gas at the temperature used. Thus 1.5 tons of water-gas at 0° centigrade has a bulk of about two thousand two hundred and thirty-two cubic meters. At 850° centigrade the same weight of gas occupies a space of eight thousand nine hundred and thirty cubic meters, and at 1,000° centigrade (which is about the temperature which I prefer to employ in my process) the same weight of gas will occupy ten thousand four hundred and fifteen cubic meters. Consequently the fan or blower is increased or reduced in size as the temperature of the gas used in the process may be high or low. In order to prevent the dilution of the reducing-gas by carbonic acid formed during and by the reduction process, the zinc ore, as stated, is preferably mixed and eventually baked with coal in about the proportions above indicated, so that during the reduction the carbonic acid is reduced *in statu nascenti* to carbon monoxid.

Any suitable apparatus can be used for carrying my improved process into effect, and approved forms of furnaces used in the reduction of other metals can be conveniently employed. Thus for the reduction of ores of relatively large size the furnace may be constructed similarly to the ordinary shaft of a lead-furnace, while for small-sized ores the furnace may be constructed upon the lines of apparatus now used for working mercury-ore dust. The furnace is provided at its top with the usual charging-hopper and with a cinder or slag door below. The twyers will be located about one-third of the height of the furnace from the bottom, and through these twyers the active reducing-gas is injected. Leading out of the furnace near its top is the eduction-pipe, made of fire-clay or of iron lined advantageously with fire-clay, the diameter of which depends, of course, upon the size of the furnace. This eduction-pipe

leads to the condensation apparatus, which may conveniently be arranged like the apparatus now used in the arts for the condensation of mercury. With a furnace of the capacity of twenty-five tons of zinc oxid or a corresponding amount of oxydic ore about five tons of the oxid will be reduced in from four and one-half to five hours, it being understood that the temperature of the water-gas injected is about 1,000° centigrade.

By the expression "oxydic ore" above used by me I mean any natural or roasted material containing zinc oxid, carbonate, silicate or hydrate, or mixtures of the same—such as roasted blende of any grade, roasted galena blende, franklinite, willemite, zincite, calamine, smithsonite, hydrozincite, &c.

I find in practice that 1.5 tons of water-gas containing 1.4 tons of carbon monoxid and .1 ton of hydrogen and occupying a bulk of ten thousand four hundred and fifteen cubic meters at 1,000° centigrade, as before stated, will be sufficient for the reduction of 8.1 tons of zinc oxid or roasted good blende or the equivalent amount of any other suitable zinc ore.

In carrying the process into effect the furnace is first charged through the hopper with the ore or mixture of ore and coal or other suitable hydrocarbon in the proportions stated, and the hot water-gas coming from the producer or gasometer and of the proper temperature is passed through the ore, carrying the zinc-vapors into the condensation apparatus. Preferably a small dust-chamber is interposed between the furnace and the condensation apparatus, in which will be collected any dust which may have become mechanically entrained and carried over with the vapors. The spelter will be condensed in the condensation apparatus at a temperature of from 415° to 550° centigrade and can be removed either from time to time or continuously, as may be desired, being received in reserve tanks or cast in suitable forms. The hot waste gases passing from the condensation apparatus being composed of carbon monoxid and hydrogen can be burned with air, and thus used for heating the ovens or for any other purpose.

While I have described my invention as being carried out in connection with a blast-furnace and as preferably utilizing an active reducing-gas in a highly-heated form, it will be understood that the reactions may take place in other forms of apparatus and that the reducing-gas need not be in a heated condition. Thus the ore may be treated in furnaces which are heated exteriorly, or, instead, the material may be heated electrically, in both of which cases the reducing-gas need not be injected into the furnace in a superheated condition. As before indicated, it will also be understood that my improved process can be carried out in connection with the condensation of zinc-vapors obtained by any other process or reaction—as, for example, by heat-

ing blende with iron or iron silicate, ( $Fe_4SiO_6$ .) It will finally be understood that zinc-vapors prepared in a blast-furnace as I have described can, if desired, be oxidized by a current of air to produce pure oxid of zinc instead of being condensed to spelter in a condensation apparatus.

I am aware that prior to my invention the use of carbon monoxid (CO) for zinc reduction had been suggested, the carbon monoxid being prepared by blowing air over coal. With such processes an objectionably large percentage of nitrogen is present, whereby the reducing-gas will be so diluted that a condensation of zinc to liquid metal is impossible. By employing water-gas, as I suggest, my zinc atmosphere contains over sixty per cent. more zinc than any carbon-monoxid atmosphere could possibly contain. My atmosphere is not only higher in concentration than in the prior processes, but has a much lower specific gravity, since hydrogen replaces the nitrogen of the other processes, thereby allowing a condensation to liquid metal.

Having now described my invention, what I claim as new, and desire to secure by Letters Patent, is as follows:

1. An improved process for condensing zinc-vapors to spelter, which consists in cooling the vapors in an atmosphere of water-gas, substantially as set forth.

2. An improved process for reducing zinc oxydic ores, which consists in subjecting the

material in the presence of heat to the reducing effect of water-gas, substantially as set forth.

3. An improved process for reducing zinc oxydic ores, which consists in subjecting the material to the reducing effect of heated water-gas, substantially as set forth.

4. An improved process of making spelter from zinc oxydic ores, which consists in subjecting the material in the presence of heat to the reducing effect of water-gas, and in cooling the resulting zinc-vapors in an atmosphere of such gas, substantially as set forth.

5. An improved process of making spelter from zinc oxydic ores, which consists in subjecting the material to the reducing effect of heated water-gas, and in cooling the resulting zinc-vapors in an atmosphere of such gas, substantially as set forth.

6. An improved process of making spelter from zinc oxydic ores or zincic materials, which consists in subjecting a mixture of such material and coal in the presence of heat to the reducing effect of water-gas, and in cooling the resulting zinc-vapors in an atmosphere of such gas, substantially as set forth.

This specification signed and witnessed this 7th day of November, 1901.

OSKAR NAGEL.

Witnesses:

FRANK L. DYER,  
JNO. ROBT. TAYLOR.